

Feb. 18, 1930.

G. R. MEYERCORD ET AL

1,747,311

METHOD OF MAKING EMBOSSED DIES

Filed March 25, 1929

2 Sheets-Sheet 1

*Fig. 1.*



*Fig. 2.*



*Fig. 3.*



*Fig. 4.*



*Fig. 5.*



Trilector  
G. R. Meyercord and  
C. B. Morris,

by W. F. Grundemich,  
atty.

Feb. 18, 1930.

G. R. MEYERCORD ET AL

1,747,311

METHOD OF MAKING EMBOSSED DIES

Filed March 25, 1929

2 Sheets-Sheet 2

Fig. 6.



Fig. 7.



Fig. 8.



Fig. 9.



Fig. 10.



By G.R. Meyercord and  
C.B. Morris,  
Mr. F. Freudenreich, *attys.*

## UNITED STATES PATENT OFFICE

GEORGE R. MEYERCORD, OF CHICAGO, ILLINOIS, AND CHARLES B. NORRIS, OF GRAND RAPIDS, MICHIGAN, ASSIGNORS TO HASKELITE MANUFACTURING CORPORATION, A CORPORATION OF NEW YORK

## METHOD OF MAKING EMBOSsing DIES

Application filed March 25, 1929. Serial No. 349,889.

The present invention relates to the art of working plywood panels so as to give them the appearance of wood carvings, and it has for its object to make possible a rapid and economical production of complementary dies, regardless of the size and character of the original subject to be re-produced, by means of which dies panels may be successfully embossed.

10 The various features of novelty whereby our invention is characterized will herein-after be pointed out with particularity in the claims; but, for a full understanding of our invention and of its objects and advantages, 15 reference may be had to the following detailed description taken in connection with the accompanying drawings, wherein:

Figure 1 is a section through a copper shell which is to form the working face of the female die; Figs. 2 and 3 are sectional views illustrating successive steps in the completion of the rudimentary female die; Fig. 4 is a plan view of the female die block positioned upon a temporary supporting plate; Fig. 5 is a section on line 5—5 of Fig. 4; Fig. 6 is a plan view of the completed female die and its holder; Fig. 7 is a section taken approximately on line 7—7 of Fig. 6; Fig. 8 is a perspective view of the cast iron case for the male die; Fig. 9 is a view partly in section and partly in elevation, showing the parts illustrated in Figs. 4 and 8 assembled preparatory to the casting of the male die; and Fig. 10 is a section through the completed male die.

In embossing a panel by pressing it between complementary dies, that die which engages the side of the panel that is to be the front or face of the latter when embossed must be sharp and distinct and be of comparatively hard material. The wood is pressed into the cavities of this die, which is the female, by the other die acting on the back of the panel. This other die, the male, while it should be a reasonable fit in the complementary die, may be made of a soft material.

We have found that electro-deposited copper possesses a sufficient degree of hardness to adapt it for use as the female die face. Therefore we begin the manufacture of the

dies by making a female die in the form of a comparatively thin copper shell 1. This shell is composed of copper electro-deposited to a thickness of about a sixteenth of an inch. The shell 1 may be produced in any suitable way. Ordinarily, a wax impression will be made of an original wood carving; a copper shell in the form of a male die will be electro-deposited upon the wax impression; this first copper shell, covered lightly with wax, dusted with graphite, may serve as a foundation upon which to electro-deposit a female copper shell. If only one set of working dies is required, this female shell may be used in the production of the working dies. However, where a plurality of similar sets of working dies are required, wax impressions may be made from the second copper shell and shells for the working female dies may be electro-deposited on these wax impressions.

Having the copper shell 1, it is placed face down in a shallow cast iron tray 2. First however, the inside of the tray and the face of the shell are painted with a paint composed of powdered graphite, zinc oxide, commercial sodium silicate, and water. Proportions that have been found to be satisfactory are as follows: graphite sixty-five grams; zinc oxide sixty-five grams; commercial sodium silicate 3 c. c.; and water 170 c. c. The graphite and the zinc oxide are mixed dry and the mixture of sodium silicate and water is then added thereto. After the shell has been placed in the tray, the edges are covered smoothly with a putty. We have found that a putty made of one part of commercial sodium silicate and nine parts of water, together with sufficient asbestos cement to give the proper consistency will serve the purpose satisfactorily. The shell is covered to a depth of about one-half inch with a flux, as indicated at 3 in Fig. 2. As a flux we have successfully employed a mixture of five parts of zinc chloride and one part of cupreous chloride. Suitable weights are then placed upon the shell to hold it down. We have illustrated a single weight 4 for this purpose. We also provide a piece of wire mesh of about the same size as the shell. A

55

60

65

70

75

80

85

90

95

100

material composed of galvanized one-eighth inch steel wire of about five-eighths inch mesh will ordinarily serve the desired purpose which is to reinforce the casting to be made in the manner now to be described.

5 A tank of molten white metal is prepared. A suitable white metal is that commercially known as Sampson metal, which is an alloy of zinc, copper and aluminum. The tank may be 10 made out of steel plate. The white metal is kept at a temperature of about 900° F. The tray and its contents, and the piece of wire mesh, are placed in the molten metal and, when the tray becomes heated to the temperature 15 of the white metal, some of the latter is ladled into the tray and the latter is then removed from the tank and permitted to cool. The weights are removed and the back of the shell is brushed lightly with a wire brush 20 to remove any small particles of flux which might adhere to it. The flux is carefully skimmed from the surface of the metal in the tray and then the piece of wire mesh is lifted out of the tank and dropped into the tray. 25 The wire mesh is pressed down until it is in contact with or at least close to the copper shell. The white metal hardens first around its edges. As soon as the edges become hard, they are clamped to the tray by means of suitable 30 clamps, such as shown at 5 in Fig. 3. The clamping of the edges of the casting prevents the casting from warping as it cools. After the casting has become cool, it is removed from the tray, the copper shell 35 adhering to it. At this point the female die has reached a stage in which it consists of a more or less rough casting 6 of white metal faced on one side with the copper shell 1 and having embedded therein a reinforcing wire 40 mesh 7.

The back of the die block is machined until it is flat, and one edge is also machined. Holes 45 8 are bored through the block at each end of the copper element, the ends of the copper element forming diameters for these holes. The block is then placed, face up, upon a plate 9 provided with stops 10 against which the finished edge of the block rests, as shown in Fig. 4. The plate is provided with dowel 50 pins 11 that extend up through the holes 8 in the die block.

The male die is made in a single operation by using the female die as a part of a mold cavity into which is poured molten metal. As 55 a foundation for the male die we employ a cast iron tray-like case 14 the top of which is depressed about a quarter of an inch or three-eighths of an inch throughout almost its entire area, leaving a comparatively narrow 60 ledge or rim 15 along the edges. From the bottom of the depression rise numerous projections 16. The flange or rim is cut away at one side and the edge of the case in this zone is beveled as indicated at 17 to produce a 65 gate into which molten metal may be poured.

The case and the female die block mounted on the temporary supporting plate 9, as in Fig. 4, are then placed face to face; the dowel pins 11 entering holes 18 in the case. A number of C-shaped stops of the kind indicated 70 at 19 in Fig. 9 are placed in position to engage the plate 9 and the back of the cast iron case. Wedges are then driven between the female die block and the case so as to spread the block and the case apart as far as the stops 75 will permit. The crack produced in what may be termed the mold by spreading the halves apart is stopped up by means of putty, as indicated at 20 in Fig. 9. A putty for this purpose that has been found to be satisfactory is one made of cylinder oil mixed with ground asbestos, that has been stored in a warm place until it has aged. Of course no putty is placed along the line of the gate. Molten zinc heated to a temperature of about 80 900° F. is then poured through the gate until the mold cavity is filled. The female die block and its supporting plate are then removed, leaving the zinc adhering to the cast iron case. The male die therefore consists of the cast 90 iron case to which is permanently united a block of zinc 21 having its face in the form of a male die.

After the female die block has been used as a pattern for the casting of the male die, the 95 three edges that remain unfinished are machined, the ends being cut off along the lines of the edges of the copper shell, cutting the holes 11 in half. The block is then set into a closely-fitting case 25, as shown in Figs. 6 100 and 7, having dowel pins 26 positioned to engage in the half holes in the female die block. Consequently, when a panel is placed between the two die blocks and the latter are brought together, the pins 26 cause the two 105 die faces to register accurately. The case into which it is fitted prevents the body of the female die block from spreading under heavy pressures; the tray 14 serving this same purpose with respect to the male die block.

While we have illustrated and described with particularity the details of the preferred method and of preferred forms of devices, we do not wish to limit ourselves to such details; but intend to cover all methods and forms of 110 construction coming within the definitions of our invention constituting the appended 115 claims.

We claim:—

1. The method of producing a die for embossing plywood in imitation of carving, 120 which consists in producing a thin copper shell having on one side the desired die face, painting said face and the inside of a cast iron tray with a material that will prevent the adherence of molten white metal, laying the shell, face down, in the tray, covering the shell with a flux, heating the tray and its contents to the temperature of molten white metal, and then pouring molten white metal 125 130

into the tray and removing the flux that rises to the top of the white metal.

2. The method of producing a die for embossing plywood in imitation of carving, which consists in producing a thin copper shell having on one side the desired die face, painting said face and the inside of a cast iron tray with a material that will prevent the adherence of molten white metal, laying the shell, face down, in the tray, covering the shell with a flux, heating the tray and its contents to the temperature of molten white metal, pouring molten white metal into the tray, and pressing down into the white metal a reinforcing member heated to about the same temperature as the white metal.

3. The method of producing a die for embossing plywood in imitation of carving, which consists in producing a copper shell having on one side the desired die face, casting a thick layer of white metal upon the back of said shell, and clamping the casting in the vicinity of its edges as soon as it has hardened at the edges, thereby to prevent warping of the casting while the center hardens.

4. The method of producing a die for embossing plywood in imitation of carving, which consists in producing a copper shell having on one side the desired die face, placing the shell face down in a cast iron tray, casting a heavy layer of white metal upon the shell, and clamping the marginal portions of the white metal casting to the tray as soon as they have become hard and before the center has hardened.

5. The method of producing a die for embossing plywood in imitation of carving, which consists in producing a copper shell having on one side the desired die face, laying the shell face down in a cast iron tray, heating the tray and its contents, pouring molten white metal into the tray, and pressing a heated piece of heavy wire mesh into the molten metal to form a reinforcement for the latter upon hardening.

6. The method of producing a die for embossing plywood in imitation of carving, which consists in producing a copper shell having on one side the desired die face, laying the shell face down in a cast iron tray, covering the shell with a flux, holding the tray in a body of molten white metal without permitting the molten metal to flow into the tray, and, when the tray and its contents have been heated to the temperature of the molten metal, lifting out the tray and pouring some of the molten white metal into the same.

7. The method of producing a die for embossing plywood in imitation of carving, which consists in producing a copper shell having on one side the desired die face, laying the shell face down in a cast iron tray, covering the shell with a flux, holding a piece of heavy wire mesh and also the tray in a

body of molten white metal without allowing the white metal to enter the tray, pouring white metal into the tray when the tray and its contents have become heated to about the temperature of the molten metal, and then placing the heated piece of wire mesh in the tray and pressing it down close to the shell.

In testimony whereof, we sign this specification.

GEORGE R. MEYERCORD.  
CHARLES B. NORRIS.

75

80

85

90

95

100

105

110

115

120

125

130